

## UNITED STATES PATENT OFFICE

2,680,123

ZINC SALT OF MIXED ESTER  
THIOPHOSPHATES

Paul K. Mulvany, Richmond, Calif., assignor to  
California Research Corporation, San Francisco, Calif., a corporation of Delaware

No Drawing. Application March 29, 1951,  
Serial No. 218,281

6 Claims. (Cl. 260—429)

1

This invention pertains to a new composition of matter prepared by reacting a mixture of two different alcohols with phosphorus pentasulfide ( $P_2S_5$ ). In particular, this invention pertains to the zinc salts of a reaction product containing mixed diesters of dithiophosphoric acids prepared by reacting phosphorus pentasulfide with a mixture of two different alcohols (one alcohol containing not more than 4 carbon atoms, and the other alcohol containing from 6 to 18 carbon atoms).

The new compositions set forth herein are useful in additives in lubricating oil compositions; particularly useful in inhibiting oxidation of lubricating oil compositions. These new compounds are remarkably effective in increasing the useful life of a lubricating oil composition which is susceptible to oxidation.

It is known that zinc salts of dialkyldithiophosphoric acids (wherein the alkyl groups are derived from the same alcohol) inhibit oxidation of lubricating oil compositions. It is also known that the alkyl groups of these zinc dialkyldithiophosphates may be of high molecular weight or low molecular weight. Zinc dialkyldithiophosphates, wherein the alkyl groups are the same and each contain less than 6 carbon atoms (e. g., 4 carbon atoms), are considerably less expensive than the zinc dialkyldithiophosphates containing alkyl groups which are the same and derived from higher molecular weight alcohols. In spite of this, these zinc dialkyldithiophosphates having alkyl groups derived from low molecular weight alcohols (e. g., alcohols of 4 carbon atoms) have not been widely marketed as lubricating oil additives. The main reason for this has been the insufficient oil solubility of the zinc salts of low molecular weight dialkyldithiophosphoric acids to be able to prepare and market a concentrate in oil. This inability to ship concentrated oil solutions of these zinc salts due to the oil insolubility at normal storage conditions has more than offset the low cost of compounds per se. The same difficulty of solubility pertains to the dialkyldithiophosphoric acids from which these zinc salts are derived.

It is a primary object of this invention to prepare dialkyldithiophosphoric acids using two unlike low molecular weight alcohols as the source of the ester groups, and the zinc salts thereof.

It is another object of this invention to prepare zinc salts of diesters of dithiophosphoric acids wherein the organo portions are derived from low molecular weight alcohols, the dithiophosphates having sufficient oil solubility to prepare concentrated solutions of the zinc salts in oil of at least 35% at  $-20^{\circ}\text{ F}$ .

2

A further object of this invention is to prepare relatively low cost mixed diesters of dithiophosphoric acids.

These and further objects of the invention will be apparent from the ensuing description and the appended claims.

It has been discovered that the products obtained by the reaction of two different alcohols with phosphorus pentasulfide, and the zinc salts thereof, possess new and unique properties.

One of the alcohols used in the reaction contains less than 4 carbon atoms. These alcohols include methyl alcohol, ethyl alcohol, propyl alcohol, isopropyl alcohol, butyl alcohol, sec-butyl alcohol and tertiary butyl alcohol. For convenience, this group of alcohols will hereinafter be called the  $R_1$  alcohols.

The other alcohol used to form the reaction product of this invention contains from 6 to 18 carbon atoms. These include the following alcohols: hexyl, methylisobutylcarbinol, ethylisopropylcarbinol, heptyl, iso-heptyl, 2-ethyl amyl, octyl, iso-octyl, 3-ethyl hexyl, 2-propyl amyl, decyl, undecyl, dodecyl, hexadecyl, octadecyl, etc.

For convenience, this group of alcohols will hereinafter be known as the  $R_2$  alcohols.

The  $R_1$  and  $R_2$  alcohols need not be present in the reaction mixture in equal molar amounts. For certain types of oils and for certain purposes it may be preferred that the mole ratio of  $R_1$  alcohols to  $R_2$  alcohols be from 1 to 5. It is particularly preferred to use a mole ratio of  $R_1$  alcohols to  $R_2$  alcohols from 2 to 4.

The reaction products of this invention are normally prepared by mixing two different alcohols, and causing the mixture of alcohols to react with phosphorus pentasulfide ( $P_2S_5$ ) at temperatures ranging from about  $120^{\circ}\text{ F}$ . to  $200^{\circ}\text{ F}$ . For example, in the preparation of a reaction

product of this invention, 4 moles of the desired alcohols (e. g., 3 moles of methyl alcohol and 1 mole of hexyl alcohol, wherein the mole ratio of methyl alcohol to hexyl alcohol is 3) are reacted with 1 mole of  $P_2S_5$  for a time sufficient to complete the esterification. The zinc salts of the reaction mixtures are prepared by reacting the dialkyl dithiophosphoric acid preparation with zinc oxide or zinc hydroxide at temperatures ranging from  $70^{\circ}\text{ F}$ . to  $170^{\circ}\text{ F}$ .

The following examples illustrate methods of preparing the new compositions of this invention.

*Example 1.—Reaction product of isopropyl alcohol, methylisobutylcarbinol and  $P_2S_5$*

A mixture of 252 parts by weight (67 mole percent) of isopropyl alcohol and 206 parts by weight

(33 mole percent) of methyl isobutylcarbinol was placed in a glass reaction vessel. To this mixture was added 333 parts by weight of  $P_2S_5$ . The whole mixture was heated at  $170^{\circ} F.$  for 2 hours, after which the reaction mixture was cooled, and the product filtered to remove a small amount of unreacted  $P_2S_5$ .

In the preparation of the zinc salt, 650 grams of the acid intermediate thus obtained was added to 130 parts by weight of a petroleum oil having a viscosity of 300 SSU at  $100^{\circ} F.$  (used as a diluent), then 122 parts by weight of zinc oxide was gradually added at  $130^{\circ} F.$  The whole mixture was then agitated for 3 hours at  $130^{\circ} F.$ , after which the water of neutralization was removed with calcium sulfate. The oil solution of the zinc salt had a pH of 6.7 (after filtration), and contained 9.96% zinc, 9.43% phosphorus and 19.42% sulfur.

*Example 2.—Reaction product of butyl alcohol, methylisobutylcarbinol and  $P_2S_5$*

A mixture of 237 parts by weight (77 mole percent) of sec-butyl alcohol and 98 parts by weight (23 mole percent) of methylisobutylcarbinol and 222 parts by weight of  $P_2S_5$  was charged to a reaction vessel and agitated at  $170^{\circ} F.$  for a period of 2 hours. The reaction mixture was cooled and filtered to remove a small amount of unreacted  $P_2S_5$ . The resulting butyl methylisobutylcarbinol dithiophosphate was a dark red green liquid having a neutralization number of 193 (mgs. KOH/gram), a viscosity of 35.7 SSU at  $100^{\circ} F.$ , a specific gravity of 1.04 (60/60), and contained 24.0% sulfur and 11.9% phosphorus.

To the above mixture was added 87 parts by weight of zinc oxide, after which the whole was heated with agitation at  $130^{\circ} F.$  for 4 hours until a pH of 6.7 was reached. After the water of neutralization had been removed, the oil solution contained 7.6% zinc, 7.2% phosphorus and 15.0% sulfur.

The oil solubility of the zinc salts of this invention wherein the two different alcohols have certain mole ratios to each other is considerably greater than zinc salts having the same mole ratio of a mixture of two diester dithiophosphoric acids (wherein the ester groups in each acid are the same; that is, each acid contains only one of the ester radicals of the above mixed diester dithiophosphoric acid). For example, a 35% petroleum oil solution of a mixture of zinc di(sec-butyl) dithiophosphate and zinc di(methylisobutylcarbinol) dithiophosphate (mole ratio of 3.35) began to crystallize from solution within a period of 2 days at  $-20^{\circ} F.$  On the other hand, an 81% oil solution (same oil as above) of the zinc salt of the reaction product prepared according to Example 2 above was still clear after 30 days at  $-20^{\circ} F.$  Similarly, an 8% petroleum oil solution of a mixture of zinc diisopropyl dithiophosphate and zinc di(methylisobutylcarbinol) dithiophosphate (mole ratio of 2) began to crystallize from solution within 3 days at  $+30^{\circ} F.$  However, an 85% petroleum oil solution of the zinc salt prepared as in above Example 1 did not show any signs of crystallization after 34 days at  $+30^{\circ} F.$

The table below presents data concerning the effectiveness of the reaction products of this invention in reducing corrosion of metal parts due to oxidation of lubricating oils during the operation of internal combustion engines. To obtain these data, a stock Chevrolet engine was used. Instead of the normal babbitt bearings of

the Chevrolet engine, two of the connecting rods were modified to accommodate copper-lead bearing inserts, which were weighed before being assembled in the engine. The Chevrolet engine was operated at 3150 R. P. M., the engine jacket temperature was maintained at  $300^{\circ} F.$ , the crankcase oil temperature was maintained at  $280^{\circ} F.$ , and the engine was operated for a period of 36 hours before being disassembled and the bearing inserts weighed. Before weighing, the bearing inserts were carefully washed with solvents to remove the oil therefrom.

*Table*

| Test No. | Oil Sample                                                                                                         | Bearing Weight Loss (Mgs./Whole Bearing) |
|----------|--------------------------------------------------------------------------------------------------------------------|------------------------------------------|
| 20       | Reference Oil for Test No. 2 <sup>a</sup>                                                                          | <sup>b</sup> 558                         |
| 2        | Reference Oil + 0.52% of the zinc salt of Example 2 above.                                                         | 36                                       |
| 3        | Reference Oil for Test Nos. 4, 5 and 6 <sup>c</sup>                                                                | 1,102                                    |
| 4        | Reference Oil + 0.81% zinc di(cetylphenyl) dithiophosphate                                                         | 50                                       |
| 5        | Reference Oil + 0.81% zinc di(cetylphenyl) dithiophosphate; + 0.091% sulfurized alkyl-substituted calcium phenate. | 344                                      |
| 25       | Reference Oil + 0.89% of the zinc salt of Example 2 above; + 0.091% sulfurized alkyl-substituted calcium phenate.  | 76                                       |

<sup>a</sup> This reference oil was a California solvent-refined paraffinic base SAE 30 oil containing 0.89% by weight of a calcium alkyl sulfonate and 0.97% by weight of a sulfurized alkyl-substituted calcium phenate.

<sup>b</sup> Weight loss after 20 hours.

<sup>c</sup> This reference oil was a Mid-Continent SAE 30 oil.

To illustrate still further the effectiveness of the reaction products of this invention as lubricating oil additives, a series of tests was run to determine the inhibition period of lubricating oils containing these reaction products. The inhibition period (the time in hours before 100 grams of oil sample utilizes 1000 cubic centimeters of oxygen at  $340^{\circ} F.$ ) of a medicinal white oil was zero hours. When 0.19% of the zinc salt of above Example 2 was added to the medicinal white oil, the inhibition period was increased to 4.2 hours.

Other uses of the zinc salts of this invention include the use as anti-oxidants in greases, anti-wear agents in silicate fluids, that is, organic esters of silicic acid, e. g., ortho silicate esters such as tetraethyl silicate, tetra(n-hexyl) silicate, tetra(2-ethylhexyl) silicate, etc.

The lubricating oils in which the new zinc salts of this invention may be incorporated include a wide variety of lubricating oils such as naphthenic base, paraffin base, and mixed base mineral oils, other hydrocarbon lubricants, e. g., lubricating oils derived from coal products and synthetic oils, e. g., alkylene polymers (such as polymers of propylene, butylene, etc., and mixtures thereof), alkylene oxide type polymers, dicarboxylic acid esters and liquid esters of acids of phosphorus. Synthetic oils of the alkylene oxide type polymer which may be used include those exemplified by alkylene oxide polymers (e. g., propylene oxide polymers) and derivatives, including alkylene oxide polymers prepared by polymerizing alkylene oxides (e. g., propylene oxide) in the presence of water or alcohols, e. g., ethyl alcohol, and esters of alkylene oxide type polymers, e. g., acetylated propylene oxide polymers prepared by acetyating the propylene oxide polymers containing hydroxyl groups.

I claim:

1. A zinc salt of mixed diesters of dithiophosphoric acids produced by reacting phosphorus pentasulfide with a blend of two different saturated aliphatic monohydric alcohols, one of said

alcohols being a lower molecular weight alcohol and containing not more than 4 carbon atoms, the other of said alcohols being a higher molecular weight alcohol and containing from 6 to 18 carbon atoms, wherein the ratio of said lower molecular weight alcohol to said higher molecular weight alcohol has a value from 1.0 to 5.0.

2. The zinc salts of mixed diesters of dithiophosphoric acids produced by reacting phosphorus pentasulfide with a blend of two different saturated aliphatic monohydric alcohols at temperatures of 120° F. to 200° F., one of said alcohols being a lower molecular weight alcohol and containing not more than 4 carbon atoms, the other of said alcohols being a higher molecular weight alcohol and containing from 6 to 18 carbon atoms, the ratio of said lower molecular weight alcohol to said higher molecular weight alcohol having a value from 2 to 4.

3. The zinc salts of the mixture of esters of 20 dithiophosphoric acids of claim 2, wherein one alcohol of the reaction blend is a butyl alcohol and the other alcohol of the reaction blend is a hexyl alcohol.

4. The zinc salts of the mixture of esters of dithiophosphoric acids of claim 2, wherein one alcohol of the reaction blend is a sec-butyl alcohol and the other alcohol of the reaction blend is a methylisobutylcarbinol.

5. The zinc salts of the mixture of esters of dithiophosphoric acids of claim 2, wherein one alcohol of the reaction blend is a propyl alcohol and the other alcohol of the reaction blend is a hexyl alcohol.

6. The zinc salts of the mixture of esters of dithiophosphoric acids of claim 2, wherein one alcohol of the reaction blend is an isopropyl alcohol and the other alcohol of the reaction blend is 15 a methylisobutylcarbinol.

References Cited in the file of this patent

UNITED STATES PATENTS

| Number    | Name                   | Date          |
|-----------|------------------------|---------------|
| 1,939,951 | Buchanan et al. ____   | Dec. 19, 1933 |
| 2,252,984 | Rutherford et al. ____ | Aug. 19, 1941 |
| 2,261,047 | Asseff et al. _____    | Oct. 28, 1941 |
| 2,368,000 | Cook et al. _____      | Jan. 23, 1945 |